

[54] PLATED WIRE MEMORY

3,354,059 11/1967 Koretzky..... 204/12  
3,370,929 2/1968 Mathias ..... 29/183.5  
3,549,507 12/1970 Semienko et al. ..... 204/28

[75] Inventor: Guy DiGuilio, Philadelphia, Pa.

[73] Assignee: Sperry Rand Corporation, Blue Bell, Pa.

[22] Filed: Apr. 22, 1974

Primary Examiner—John H. Mack

[21] Appl. No.: 463,002

Assistant Examiner—Aaron Weisstuch

Attorney, Agent, or Firm—Rene A. Kuypers

Related U.S. Application Data

[62] Division of Ser. No. 375,266, June 29, 1973, Pat. No. 3,853,717.

[57] ABSTRACT

[52] U.S. Cl. .... 29/191.6; 29/196; 29/196.3; 29/199; 340/174 PW; 75/170

There is disclosed herein a quaternary alloy plating composition for a NDRO (non-destructive read-out) magnetic memory wire comprising by weight 77.3% Ni, 18.2% Fe, 3.5% Co, 1.0% P and substantially non-magnetostrictive.

[51] Int. Cl. ... B23p 3/00; G11c 11/02; C22c 19/00

[58] Field of Search ..... 204/12, 13, 28, 43 T, 43 P; 340/174 PW; 29/196, 196.3

[56] References Cited

UNITED STATES PATENTS

3,330,631 7/1967 Tsu ..... 29/183.5

5 Claims, 5 Drawing Figures



Fig. 1



Fig. 3



Fig. 4

## PLATED WIRE MEMORY

This is a division of application Ser. No. 375,266, filed June 29, 1973, now U.S. Pat. No. 3,853,717.

## BACKGROUND OF THE INVENTION

## 1. Field of the Invention

This invention relates to the field of computer memories and in particular to the magnetic type that operates in the NDRO mode.

## 2. Description of the Prior Art

The known pertinent prior art is contained in the IEEE Transactions on Magnetics, Vol. Mag.-5, No. 4, December, 1969, pp. 728-751 by J. S. Mathias and G. A. Fedde, and U.S. Pat. Nos. 3,370,929 and 3,549,507.

The recognized shortcoming of the known prior art plated wires has been their narrow operating margins. This means that the plated wires with such operating characteristics are able to withstand only limited current variations along the bit and word lines. This is a serious shortcoming since such wires are rejected during the manufacturing process and therefore the production yields are decreased and the unit cost increased. In other words, plated wires manufactured with limited operating margins make it difficult to compete in the marketplace and hence, are not viable memory devices.

The instant invention is designed to provide a NDRO plated wire memory element with a wider range of magnetic characteristics than exists in the prior art. In particular, the present invention provides wires having an increased wall motion threshold. The wall motion threshold is the upper limit of bit current (current down the wire in the write mode) allowed in the operation of the plated wire. If the wall motion threshold is exceeded, information stored along the wire will be destroyed.

The present invention also is designed to provide a higher degree of uniformity along the length of the wire and a larger operating region so that better utilization of the wire can be obtained. By uniformity is meant that the magnetic parameters of the wire have reduced variations along the length of the wire.

The gist of the invention is accordingly a new magnetic plating composition composed of nickel, iron, cobalt and phosphorus on a uniformly rough or spherular, hereinafter referred to as caviar intermediate layer. The caviar surface is formed on a smooth, mirror-like, non-magnetic wire substrate.

## BRIEF DESCRIPTION OF THE DRAWINGS

FIG. 1 is a schematic representation of the plating process utilized in the invention;

FIG. 2 depicts in schematic form the various currents applied during the plating process as well as a schematic of the cell arrangement which is utilized;

FIG. 3 is a view of a smooth, drawn wire as initially provided during the plating operation at 3,000 magnification wherein 3 millimeters thereon equal 1 micron (~0.00004 in.)

FIG. 4 is a view of the uniformly rough or intermediate surface plated upon the substrate shown in FIG. 3 at 3,000 magnification wherein 3 millimeters thereon equals 1 micron; and

FIG. 5 depicts a simplified switching diagram of a bit along the plated wire provided by the present invention as well as for the prior art plated wire.

## DESCRIPTION OF THE PREFERRED EMBODIMENTS

Referring now to FIG. 1 in greater detail, there is shown a reel 10 having several feet of wire substrate 11 wound around its circumference. The substrate 11 is made of non-magnetic material such as beryllium-copper or phosphor-bronze alloy on the order of about 2-5 mils in diameter. Prior to placing the substrate 11 on the reel 10, it may be electropolished in accordance with well established prior art practices to remove troublesome defects such as die marks, gouges and inclusions, refractory oxides, etc.

As the plater arrangement shown in FIG. 1 is placed in operation, the smooth substrate 11 is first electro-cleaned at station 12 in order to remove grease, dirt and extraneous matter. Well established prior art materials and procedure are utilized during this step of the operation. The schematic shown in FIG. 2 indicates that during the electrocleaning step, current (see Table III) is supplied to the cell between the anode and cathode. The actual cell construction will be discussed in greater detail hereinafter. As is readily understood, the electrical current path is provided through the anode connection, the electrolyte, the substrate 11 to the cathode connection or ground. Following the electrocleaning operation, the substrate 11 is rinsed at station 14', following which it is subjected to an acid etch at station 16 and further rinsed at station 14". The acid etch is utilized to dissolve any residual metallic oxides still remaining on the substrate after the electroclean step.

Following electrocleaning, acid etch and water rinses, the substrate 11 is subjected to a copper plating operation at station 18. The purpose of the copper plating is to provide a uniformly rough (as opposed to a randomly rough) surface on the smooth wire substrate. This surface has been described as nodular or caviar and is shown in magnified form in FIG. 4. The nodular copper surface is typically plated to a thickness of approximately 5-10,000 Å. The copper can be deposited from a pyrophosphate copper solution, or preferably from a high-efficiency cyanide bath of the composition given in Table I.

TABLE I

|                           | Range      | Preferred |
|---------------------------|------------|-----------|
| Copper Cyanide (g)        | 50-62      | 56        |
| Potassium Cyanide (g)     | 87-108     | 92        |
| Water (l)                 | 1          | 1         |
| Copper as metal (g)       | 36/44      | 40        |
| Free Cyanide as KCN (g)   | 5-17.5     | 11.5      |
| Ratio Cu/KCN              | 2.5 to 7.5 | 3.5       |
| pH                        | 9.6-10.0   | 9.8       |
| Substrate diameter (mils) | 2½-5       | 2½-5      |

It should be noted that the pH can be adjusted with KOH.

In the instant invention, the cyanide solution is preferred. Referring again to FIG. 2, there is shown in schematic form the electrical connection for the copper deposition step. The current parameters applied during this step of the operation are shown in Table III.

After rinsing the substrate 11 at station 14", the nodular covered wire is subjected to a magnetic plating process at station 20. Formulations for useful Permalloy electrolytes are given in Table II below.

TABLE II

|                                                     | Range        | Preferred |
|-----------------------------------------------------|--------------|-----------|
| Nickel Sulfamate (g)                                | 290-350      | 320       |
| Ferrous Sulfamate (g)                               | 5.0-6.2      | 5.6       |
| CoSO <sub>4</sub> ·7H <sub>2</sub> O (g)            | 1.0-2.5      | 1.5       |
| Boric Acid (g)                                      | 20-40        | 25        |
| Trisodium Salt of Naphthalene tri-sulfonic acid (g) | 10-20        | 16.5      |
| Water (l)                                           | 1            | 1         |
| Sulfamic acid (g)                                   | 2-4          | 3         |
| pH at 23°C                                          | 2.0-3.0      | 2.4       |
| Ratio Ni/Fe                                         | 50/1 to 70/1 | 60/1      |
| Sodium Hypophosphite (g)                            | 0.04-0.20    | 0.08      |
| Temp. (°C)                                          | 50-60        | 53        |
| Substrate diameter (mils)                           | 2½-5         | 2½-5      |

The film is deposited at a thickness of between 4K-7K Å. The resulting magnetic film deposited on the uniformly rough surface would analyze by weight in the range of about 76-80% Ni, 17-18% Fe, 2-5% Co and 0.5-2.0% P with the composition nonmagnetostrictive. Non-magnetostrictive wire is an important property for plated wire manufacture because of its mechanical flexibility. In the event that the wire were made with positive or negative magnetostriction, torsion would cause large changes in its magnetic behavior.

The cell construction utilized at stations 12, 16, 18 and 20 is fully disclosed in U.S. Pat. No. 3,682,185. The cell disclosed therein is designed to maintain compositional uniformity and thickness along the length of the wire and around the circumference at stations 18 and 20. In the present invention, the plating cell is 2-3 inches across, however, the length of the active plating chamber is approximately 1¼ inches. It should be noted hereat that although one magnetic plating cell is shown in FIG. 1, several cells may be utilized. The number of cells used is a function of the plating speed and in the preferred embodiment of 14 inches/min., two cells are utilized at the respective stations 18 and 20.

Referring again to FIG. 2, the bias current is shown as flowing through the wire in addition to the electro-clean, copper deposition and magnetic plating currents. The bias current is utilized to orient the magnetization of the magnetic film circumferentially around the wire. In this situation, the circumferential direction is known as the EASY axis direction. A direction 90° removed from the EASY direction is known as the HARD direction. During the write or read cycle of the plated wire memory, the magnetization is rotated to some angle less than 90°. Suitable conditions for plating upon substrates are described in Table III below.

TABLE III

|                                         | 2½ MIL WIRE                    |           | 5 MIL WIRE                      |           |
|-----------------------------------------|--------------------------------|-----------|---------------------------------|-----------|
|                                         | Range                          | Preferred | Range                           | Preferred |
| Cleaner Current (ma/cm <sup>2</sup> )   | 800-2400                       | 1600      | 400-1200                        | 800       |
| Cleaner Temp. (°C)                      | 50-70                          | 60        | 50-70° C                        | 60        |
| Copper Current (ma/cm <sup>2</sup> )    | 160-1900                       | 900       | 80-1200                         | 900       |
| Copper Temp. (°C)                       | 25°-45°                        | 35        | 25-45                           | 35        |
| Copper Flow (M/min)                     | 300-600                        | 450       | 300-600                         | 450       |
| Permalloy Current (ma/cm <sup>2</sup> ) | For 8-16ma per cell<br>130-260 | 190       | For 22-36ma per cell<br>170-300 | 220       |
| Temp. (°C)                              | 50-60                          | 53        | 50-60                           | 53        |
| Flow (ml/min)                           | 600-1000                       | 800       | 600-1000                        | 800       |
| Annealing Temp. (°C)                    | 300-370                        | 350       | 330-370                         | 350       |
| Wire Speed (in/min)                     | 12-22                          | 14        | 12-22                           | 14        |
| Bias Current (ma)                       | 100-400                        | 300       | 600-900                         | 750       |

Referring now to the plated wire switching diagram of FIG. 5, the bit current is shown as the abscissa and the word current is shown as the ordinate. As is understood in the art, the bit current is the current applied down the plated wire during a write cycle, whereas the word current is applied to the strap positioned orthogonal to the plated wire. The word strap is energized at the same time as the plated wire is energized for a write cycle, whereas the word strap alone is energized during a read cycle. The single write switching threshold output is the locus of coincident word and bit currents which are required to write so that a certain output level is achieved on reading with the same word current. The upper limit of the word current shown on FIG. 5 is where the DRO (destructive read-out) is obtained and is produced by exceeding the NDRO limit of the wire. The upper limit of the bit current is set by the wall motion threshold and is the level of bit current where the domain walls between oppositely magnetized bits move along the wire under the influence of the bit field. Such wall motion will cause magnetization reversal of some bits along the wire and loss of information. The operating margin for a write cycle is the difference between the Bit Current Disturb Line (bit disturbance caused by the bit current alone) and the single write threshold curve. The operating point of the memory at any given level of word current must lie between these limits. The operating "window" in which the operating point may lie must also be located between the two curves.

In the prior art plated wire manufacture, the width of the margin between the single write threshold and the Bit Current Disturb line has been relatively narrow. This margin is shown as a difference between the prior art single write threshold curve (dotted line) and the Bit Current Disturb. Therefore, in the prior art, these curves have not been sufficiently separated and the operating "window" has been small. Accordingly, plated wires made in accordance with the prior art technique have a low manufacturing yield because in many wires the bit current operating margin shown in FIG. 5 is smaller than that which is required for memory operation.

Moreover, it has been the desire of those skilled in the art to make the limits of the single write threshold and the Bit Current Disturb further apart so that the required operating window becomes even larger. The instant invention has provided a larger window by effec-

tively moving the single write threshold curve further to the left (i.e., the solid curve line). This has opened up the margin between the two curves shown in FIG. 5 and as a result higher production yield is attained as well as better utilization of the wire. Thus, the wires made in accordance with the invention have larger operating margin so that they can withstand a greater variation in the circuitry connected to the word strap and the bit line. In other words, even though the circuitry connected to the plated wire memory degrades due to age and as a result of other variables so that the operating point shifts, nevertheless the wire will continue to operate satisfactorily because of the greater operating window provided.

Another improvement obtained by the present invention has been the greater uniformity of magnetic properties along the length of the wire and may be appreciated by referring to FIG. 5. FIG. 5 depicts the magnetic properties of a single bit. It has been found that the magnetic characteristic of the bits along the wire have in general the same locus of points as the bit depicted, thereby providing a high degree of uniformity in terms of wire characteristics as a function of the bit position along the wire.

What is claimed is:

1. An improved plated wire memory device having a

smooth non-magnetic wire substrate of the group consisting of beryllium-copper and phosphor bronze, a nodular intermediate layer of copper, the improvement comprising:

- a. a magnetic film deposited upon said intermediate layer comprising by weight in the range of about 17-18% Fe, 2-5% Co and 0.5-2.0% P and the balance essentially nickel,
  - b. whereby said memory is operative in the NDRO mode, and
  - c. said film being substantially non-magnetostrictive.
2. A plated wire memory device in accordance with claim 1 wherein said wire substrate has a diameter of about 2-10 mils.
3. A plated wire memory device in accordance with claim 1 wherein said magnetic film has a thickness of about 4K-7K Å.
4. A plated wire memory device in accordance with claim 1 wherein said intermediate layer has a thickness of about 5,000-10,000 Å.
5. A plated wire memory device in accordance with claim 1 wherein said magnetic film is deposited with a circumferential EASY axis.